

W. A. HALL.  
LIQUID FUEL.  
APPLICATION FILED MAY 6, 1915.

1,239,100.

Patented Sept. 4, 1917.



# UNITED STATES PATENT OFFICE.

WILLIAM A. HALL, OF NEW YORK, N. Y.

## LIQUID FUEL.

1,239,100.

Specification of Letters Patent. Patented Sept. 4, 1917.

Application filed May 6, 1915. Serial No. 26,395.

To all whom it may concern:

Be it known that I, WILLIAM AUGUSTUS HALL, a citizen of the United States of America, and residing at New York city, New York, United States of America, have invented a certain new and useful Improvement in Liquid Fuel, of which the following is a specification.

The subject of this invention is a new hydrocarbon liquid fuel suitable for use in high speed internal combustion engines and possessing the desirable qualities of both benzol and petrol. The new product is a slow burning fuel yet has as low an initial boiling point as ordinary gasolene and as large or larger fractions volatile at low temperature (say below 80° C.). It is substantially free from liability to pre-ignite and therefore in an engine using the fuel knocking does not occur even with the spark advanced. As a direct result there is much less wear and tear on the engine, and the engine can be operated while under full load at lower engine speed or on a higher gear than when run on ordinary gasolene, which means a considerable saving in fuel consumption, less frequent changing of gears and slipping of clutches. Such fuel has been found particularly advantageous for use in commercial vehicles and in city traffic where frequent stopping and starting is required. The new fuel produced in the manner hereinafter described can be "cut" at a higher temperature than can ordinary gasolene—it can be "cut" say at 180° C., as compared with 160° C. in the case of an ordinary gasolene. Its larger fractions volatile at low temperature have been found to carry complete combustion to the fractions volatile only at the highest temperatures, a considerably increased mileage per gallon consumed being the result.

The low flash point and low initial boiling point give in an engine run on the fuel great ease in starting in cold weather, and owing to its large fractions volatile at low temperatures great flexibility and quickness of acceleration is obtained. It has been found that as great flexibility and ease of starting can be obtained with this fuel when "cut" at 180° C., and of specific gravity 0.760, as can be obtained on gasolene of specific gravity 0.730 "cut" at 160° C.

A distinguishing characteristic of the new fuel is that it contains a proportion of unsaturated hydrocarbons which proportion will naturally vary with the oil

used in its production and with the details of the operation. It contains a large percentage of hydrocarbons of the ethylene series but is nevertheless quite free from the objectionable features ordinarily inherent in products containing more than a small percentage of such hydrocarbons.

The fuel having these peculiar and highly valuable properties may be produced by an endothermic chemical reaction between a gas which would be permanent under ordinary conditions of temperature and pressure, and a vapor of a hydrocarbon spirit, which vapor, if condensed to a liquid in the customary manner at atmospheric temperature, would not answer the purpose of a satisfactory motor fuel, the combination of the permanent gas and vapor being effected by mechanical compression while at a temperature sufficiently high to maintain said hydrocarbon spirit largely or wholly in the vapor state.

The new liquid fuel may be compared and contrasted with petrol as follows:—

The new fuel possesses an abnormally high specific gravity in accordance with its boiling points as distinguished from petrol and can be nitrated in the same manner as benzol. The fact that this material can be nitrated, by treating the same with nitric acid, shows that it contains considerable proportions of aromatic hydrocarbons.

In one example it has a specific gravity of about .767, yet on fractionation has an initial boiling point of about 33° C., all boiling below 150° C., 60% boiling below 100° C.; a straight gasolene distillate having such fractionation would have a specific gravity of about .70.

The new fuel readily nitrates, due to the presence of aromatic hydrocarbons combining with its own weight or more of nitric acid and in this respect, differing from petrol which does not nitrate.

The odor of the new fuel when fully refined is quite different from that of petrol or gasolene.

The new fuel is also characterized by having a much greater vapor tension.

When a very little acid is added to the new fuel, a sweet aromatic odor is produced.

The new fuel contains a certain amount of the aromatic series of hydrocarbons, (benzol and toluol); it always contains a certain amount of unsaturated hydrocarbons (or hydrocarbons of the ethylene series, and some hydrocarbons more unsaturated

than the ethylenes) varying between 20 and 50% and its iodin and bromin numbers are in accordance therewith.

The new fuel may be distinguished from 5 gasoline by the following mode of identification:—If a natural gasolene distillate that is practically all saturated, such as Pratt's perfection spirit and standard shell spirit, be mixed with denatured ethyl alcohol half 10 and half, then approximately  $\frac{1}{2}$  of this mixture will be found that is miscible and  $\frac{1}{2}$  will remain uncombined, non-miscible. Substantially the same result is obtained when 15 the new fuel is so treated, but if the unsaturated portions of the new fuel be separated and taken off by sulfuric acid absorption and the saturated portions, after being washed and refined, be mixed with alcohol, the saturated portion will not be at all miscible either in ethyl alcohol or methyl alcohol.

This spirit has a higher calorific value than gasoline and will give about 15% more miles per gallon in the average motor 25 car.

Another characteristic is that it will evaporate more rapidly than gasoline or even than benzol.

The fuel has a composition of approximately 30 85.9% of carbon and 12.76% of hydrogen, corresponding to a carbon to hydrogen ratio of 6.73 to 1, the carbon being in excess of that required by either the saturated or ethylene series of hydrocarbons due 35 to the presence of aromatic and acetylene hydrocarbons. The liquid yields, when distilled up to 150° C., more or less of gases and vapors uncondensed by ordinary water cooling, these gases containing about 26.6% of 40 unsaturated hydrocarbons. When this gas is treated with fuming sulfuric acid, then mixed with oxygen and exploded, carbon dioxid and water vapor in the ratio of 3 to 4 (by weight) are produced, and the gas with- 45 out the sulfuric acid treatment, when being mixed with oxygen and exploded giving carbon dioxid and water vapor in the ratio of 5 to 4.1.

The following table indicates in detail the 50 fractions of the new fuel boiling at temperatures differing by 10° C.

| Sp. Gr. .767  | I. B. P. 33° C. |
|---------------|-----------------|
| Boiling up to | 50° C. 2 %      |
| " " "         | 60 10 %         |
| " " "         | 70 22 %         |
| " " "         | 80 35 %         |
| " " "         | 90 55 %         |
| " " "         | 100 61 %        |
| " " "         | 110 71.5 %      |
| " " "         | 120 82 %        |
| " " "         | 130 89 %        |
| " " "         | 140 95 %        |
| " " "         | 150 All over.   |

I call attention particularly to the very 65 large amounts of material volatile at temperatures between 80 and 100° C., as shown in the above table.

The new fuel may be produced from paraffin mineral oil by a process consisting of 70 the following steps:

(1) Cracking an oil—(which may be crude, "gas", fuel, lamp or almost any distillate that in itself has a range of boiling temperatures that would not permit its use as 75 a fuel in the ordinary automobile engine)—in a continuous tube of small size (1 to 3 inches in diameter) and of sufficient length, at an average temperature of from 540° C. to 600° C. on the exterior of the tube and under pressure preferably of about 75 lbs. per square inch, with a speed of flow of oil in the pipe regulated to produce a maximum of cracking with a minimum of fixed or permanent gas consistent with economy of operation.

(2) Expanding the product subsequent to the cracking operation by reducing the pressure.

(3) Cooling the vapors and gases when in 90 this expanded state and from them separating such portions as condense below the point at which the "cut" is to be made—usually from 180° C. to 200° C.

(4) Producing an endothermic chemical 95 reaction between the gas and vapors by compressing in a mechanical compressor to a pressure preferably from 100 to 125 lbs. per square inch all the gas that has been produced along with all the vapors that boil below the temperature of the "cut", admitting these into the cylinder of the compressor at a temperature sufficiently high that they enter while in the state of vapor and mist, the fixed gas that has not been attached being permitted to separate after cooling under pressure, subsequent to the mechanical compression and be collected for other use.

(5) Clarifying and deodorizing the product 110 by extracting the yellow resinous colloidal matter which it contains, preferably by distilling it in the presence of a small amount of fullers' earth.

The process herein described may be carried out in an apparatus such as is shown in the accompanying drawing. In said drawing oil is forced by the pump 1, through the superheating coil 2, heating coil 4, located in a space 3, heated by burners 5. 6 is a pyrometer placed between the coils of the pipe 4. The gases and vapors pass by pipe 7 past the pressure-regulating valve 8, into a first cooler 9, surrounded by a cooling jacket 10, and filled if desired with a suitable filling material 11, and any heavy condensate collected therein being drawn off through pipe 12. The gases and uncondensed vapors flow by pipe 13 to a second

similar cooler 14, in which a light condensate may separate out, which may be drawn off through pipe 15, to be again introduced from pump 1 into the heating coils.

5 The gases and vapors leaving the upper part of the tower 14, for example at a temperature of 180 to 200° C., pass through a trap 16, wherein a portion of the mist carried by the gases may separate out, and be returned 10 to the tower 14 by means of the pipe 16\*. The gases and vapors are then compressed in the pump 17, wherein the endothermic reaction takes place, and are passed by pipe 18 to condensers 19 and 20, the condensate 15 collecting in tank 21, and the uncondensed gas escapes through the pipe 22.

In my copending application 26,546, I have described and claimed a crude motor fuel, produced in accordance with the process described herein, certain of the claims 20 of said application being broad enough to cover also the refined fuel.

This application is in part a continuation of my copending applications as follows:

25 Serial No. 824,194—filed March 12, 1914,

Serial No. 829,634—filed April 6, 1914,

Serial No. 3,955—filed January 23, 1915, in which applications I have claimed the process described in the present application.

30 I do not herein claim the process and apparatus herein described, the same being claimed in the cases above enumerated, and in my Patent 1,175,909 and in my copending application 77,375 filed February 9, 35 1916.

I claim:

1. A water-white liquid fuel having the composition when analyzed of approximately carbon 85.9%, hydrogen 12.76%, 40 having a carbon to hydrogen ratio of about 6.73 to 1, said fuel having a specific gravity of not materially below .76, a materially larger percentage of the same being volatile at 100° C., than would be the case with 45 ordinary gasoline, said fuel containing ethylene hydrocarbons and aromatic hydrocarbons, said fuel being further characterized by the properties of slow burning, rapid ignition, having flash point and initial boil- 50 ing point at least as low as those of ordinary gasoline and high bromin absorption value, said fuel being substantially free from yellowish, resinous, colloidal matter.

2. A refined liquid fuel having approximately the composition when analyzed of carbon 85.9, hydrogen 12.76, a carbon-hydrogen ratio of 6.73 to 1, the carbon being in excess of that required by either the saturated or ethylene series, said fuel being 55 substantially free from yellowish, resinous, colloidal matter.

3. A motor fuel which when treated with

sulfuric acid in amount sufficient to remove the unsaturated portions, leaves a saturated liquid substantially all of which is immiscible with either methyl alcohol or ethyl alcohol, said fuel containing aromatic hydrocarbons, open-chain saturated hydrocarbons, and open-chain unsaturated hydrocarbons.

4. A liquid fuel having about 35% volatile at 80° C., and a specific gravity of not less than .76, having an initial boiling point at least as low as that of ordinary gasoline, said fuel being substantially free from resinous matter, said fuel containing aromatic hydrocarbons, open-chain saturated hydrocarbons, and open-chain unsaturated hydrocarbons.

5. A liquid fuel having a gravity not below .76, about 35% thereof being volatile 80 at 80° C., said fuel being free from yellowish, colloidal, resinous matter, said fuel containing aromatic hydrocarbons, open-chain saturated hydrocarbons, and open-chain unsaturated hydrocarbons.

6. A refined motor fuel characterized by the properties of slow burning, and rapid ignition, said fuel having flash point and initial boiling point at least as low as those of ordinary gasoline, having fractions volatile at 80° C., and at 100° C., at least as large as those of ordinary gasoline, said fuel being substantially free from yellowish, resinous, colloidal matter, said fuel containing aromatic hydrocarbons, open-chain 95 saturated hydrocarbons, and open-chain unsaturated hydrocarbons.

7. A water-white motor fuel containing considerable quantities of unsaturated hydrocarbons, said fuel having an initial boiling 100 point below 35° C., having a specific gravity of not less than .76, and having materially larger fractions volatile at 100° C., than would be the case with ordinary gasoline, said fuel being substantially free from yellow, resinous, colloidal matter, and having a carbon to hydrogen ratio of about 6.73:1.

8. A water-white motor fuel suitable for use in internal combustion engines having 110 a specific gravity not materially below .76, and having a carbon to hydrogen ratio of 6.73 to 1, said fuel being substantially free from yellowish, resinous, colloidal matter.

9. A water-white motor fuel having a 115 gravity of about .76, having as much as 35% volatile at 80° C., all of said fuel distilling below 150° C., said fuel being substantially free from yellowish, resinous, colloidal matter, said fuel containing aromatic hydrocarbons, open-chain saturated hydrocarbons, and open-chain unsaturated hydrocarbons.

10. A water-white hydrocarbon product

4  
having a gravity not materially below .76, containing olefin hydrocarbons and open-chain hydrocarbons more unsaturated than the olefins, said fuel being substantially free from yellowish, resinous, colloidal matter, and not materially less than 35% of said fuel being volatile at 80° C.

11. A liquid hydrocarbon motor fuel, having a gravity of not less than .76, and 10 containing aromatic hydrocarbons, olefin hydrocarbons and hydrocarbons more unsaturated than olefin hydrocarbons, not less than about 35% of said fuel being volatile at 80° C., and not less than about 61% 15 of said fuel being volatile at 100° C., said fuel having a carbon to hydrogen ratio of about 6.73 to 1, and having a higher calorific value than ordinary gasoline, said fuel being substantially free from yellowish, 20 resinous, colloidal matter.

12. A substantially water-white motor fuel consisting essentially of hydrocarbons, and containing aromatic hydrocarbons, olefin hydrocarbons and hydrocarbons more 25 unsaturated than the olefins, said fuel having a gravity of not less than about .76, said fuel being substantially free from yellowish, colloidal, resinous matter, and having a carbon to hydrogen ratio of substantially 6.73:1.

13. A motor fuel, having a boiling point range of at least from 33° C. to 140° C., being substantially water white, free from colloidal, resinous, yellowish matter in solution, and having a carbon to hydrogen ratio of about 6.73 to 1.

14. A water-white motor fuel containing ethylene hydrocarbons, aromatic hydrocarbons, and open-chain hydrocarbons more 40 unsaturated than olefin hydrocarbons, not less than about 60% of said fuel being volatile at 100° C., said fuel being substantially free from yellowish, colloidal, resinous matter.

45 15. A motor fuel of a gravity of over .76 of which not less than about 61% is volatile at 100° C., said fuel being substantially free from yellowish, colloidal, resinous matter.

16. A motor fuel having substantially the following fractionation table:

|               |                           |      |   |
|---------------|---------------------------|------|---|
| Boiling up to | 50° C                     | 2    | % |
| " "           | 60° C                     | 10   | % |
| " "           | 70° C                     | 22   | % |
| " "           | 80° C                     | 35   | % |
| " "           | 90° C                     | 55   | % |
| " "           | 100° C                    | 61   | % |
| " "           | 110° C                    | 71.5 | % |
| " "           | 120° C                    | 82   | % |
| " "           | 130° C                    | 89   | % |
| " "           | 140° C                    | 95   | % |
| " "           | 150° C, substantially all |      |   |

said product being free from resinous coloring matter, substantially as described.

17. A water-white motor fuel having a 65 gravity of .76, of which about 35% is volatile at 80° C., and about 61% is volatile at 100° C., said fuel being substantially free from yellowish, resinous, colloidal matter.

18. A motor fuel having a gravity of .76, 70 containing between about 20% and about 50% of unsaturated hydrocarbons and having not less than about 35% volatile at about 80° C.

19. A motor fuel having substantially the 75 following fractionation table:

|               |                           |      |   |
|---------------|---------------------------|------|---|
| Boiling up to | 50° C                     | 2    | % |
| " "           | 60° C                     | 10   | % |
| " "           | 70° C                     | 22   | % |
| " "           | 80° C                     | 35   | % |
| " "           | 90° C                     | 55   | % |
| " "           | 100° C                    | 61   | % |
| " "           | 110° C                    | 71.5 | % |
| " "           | 120° C                    | 82   | % |
| " "           | 130° C                    | 89   | % |
| " "           | 140° C                    | 95   | % |
| " "           | 150° C, substantially all |      |   |

In testimony whereof I have signed my name to this specification in the presence of 90 two subscribing witnesses.

WILLIAM A. HALL.

Witnesses:

H. D. JAMESON,  
HAROLD E. C. FAIRWEATHER.